# EUROPEAN PATENT SPECIFICATION

(11) **EP 1 390 171 B1**
(45) Date of publication and mention of the grant of the patent: **10.11.2004**
(21) Application number: 02723031.7
(22) Date of filing: 17.04.2002
(51) Int. Cl.: B22F 3/00, C10M 105/68, C10M 171/06

(54) **IRON POWDER COMPOSITION INCLUDING AN AMIDE TYPE LUBRICANT AND A METHOD TO PREPARE IT**
EISENPULVERZUSAMMENSETZUNG MIT EINEM AMID-SCHMIERMITTEL UND VERFAHREN ZU IHRER HERSTELLUNG
COMPOSITION DE POUDRE DE FER CONTENANT UN LUBRIFIANT DU TYPE AMIDE ET SON PROCEDE DE PREPARATION

(30) Priority: 17.04.2001 SE 0101344
(43) Date of publication of application: 25.02.2004
(73) Proprietor: HÖGANÄS AB, 263 83 Höganäs (SE)
(72) Inventor: VIDARSSON, Hilmar, S-263 53 Höganäs (SE); KNUTSSON, Per, S-262 43 Ängelholm (SE)
(74) Representative: Thylén, Eva Matilda
(86) International application number: PCT/SE2002/000762
(87) International publication number: WO 2002/083345

(56) References cited:
- US-A- 5 368 630
- US-A- 5 744 433
- PATENT ABSTRACTS OF JAPAN & JP 04 136 104 A (HITACHI POWDERED METALS CO LTD) 26 August 1992

## Description

### FIELD OF THE INVENTION

The present invention relates to metal powder compositions. Particularly the invention relates to iron-based compositions suitable for compaction at elevated temperatures.

### BACKGROUND OF THE INVENTION

The powder metallurgy art generally uses different standard temperature regimes for the compaction of a metal powder to form a metal component. These include chill-pressing (pressing below ambient temperatures), cold-pressing (pressing at ambient temperatures), hot-pressing (pressing at temperatures above those at which the metal powder is capable of retaining work-hardening), and warm-pressing (pressing at temperatures between cold-pressing and hot-pressing).

Distinct advantages arise by pressing at temperatures above ambient temperature. The tensile strength and work hardening rate of most metals is reduced with increasing temperatures, and improved density and strength can be attained at lower compaction pressures. The extremely elevated temperatures of hot-pressing, however, introduce processing problems and accelerate wear of the dies. Therefore, current efforts are being directed towards the development of metal compositions suitable for warm-pressing processes.

The US patent 4,955,789 (Musella) describes warm compaction in general. According to this patent, lubricants generally used for cold compaction, e.g. zinc stearate, can be used for warm compaction as well. In practice, however, it has proved impossible to use zinc stearate or ethylene bisstearamide (commercially available as ACRAWAX®.), which at present are the lubricants most frequently used for cold compaction, for warm compaction. The problems, which arise, are due to difficulties in filling the die in a satisfactory manner.

The US patents 5,744,433 (Storstrom et al) and 5,154,881 (Rutz) disclose metal powder compositions including amide lubricants, which are especially developed for warm compaction.

The lubricant according to the US patent 5,744,433 contains an oligomer of amide type, which has a weight-average molecular weight M_{w} of 30,000 at the most. Very high densities and green strengths may be obtained by warm compacting powder compositions when the lubricant has a molecular weight above 4000, the preferred lubricant molecule having a molecular weight of about 6500. It has however been found that this lubricant has a tendency of sticking to the die wall, which requires frequent cleaning of the die. Another disadvantage is that the obtained green bodies are stained.

In the US. Patent 5,154,881 the amide lubricant consists of the reaction product of a monocarboxylic acid, a dicarboxylic acid and a diamine. The only lubricant tested according to this patent is ADVAWAX® 450, the composition of which is not described in detail but the reaction product obtained includes i.a. ethylene bisstearamide according to Chemis-CIVS. Our experience of this product is that it is difficult to obtain a constant composition and quality, which in turn may result in components of varying quality. This may cause problems when the lubricant is used in large scale industrial production.

### OBJECTS OF THE INVENTION

An object of the present invention is to reduce or eliminate current problems associated with large scale production.

A second object is to provide a new type of lubricant useful in metal compositions intended for compaction at elevated temperatures.

A third object is to provide a metal powder for producing components without stains.

A fourth object is to provide a metal composition including lubricant, which during the compaction of the metal powder does not deposit on the die wall.

### SUMMARY OF THE INVENTION

These objects are achieved by using a powder composition comprising an iron-based powder and new oligomer amide type lubricant. The composition may also include one or more additives, such as binders, flow agents, processing aids and hard phases.

The warm compaction may be performed by mixing an iron-based powder with the oligomer amide type lubricant and optionally a binder, preheating the powder composition and compacting the metal-powder composition in a pre-heated tool.

### DETAILED DESCRIPTION OF THE INVENTION

The new amide type lubricant used according to the present invention may be represented by the following formula

D-Cₘₐ-B-A-B-C_{mb}-D

wherein
D is -H, COR, CNHR, wherein R is a straight or branched aliphatic or aromatic group including 2-21 C atoms
C is the group -NH (CH₂)ₙCO-
B is amino or carbonyl
A is alkylen having 4-16 C atoms optionally including up to 4 O atoms
ma is an integer 1-10
mb is an integer 1-10
n is an integer 5-11.

It is preferred that D is COR, wherein R is an aliphatic group 16 - 20 C atoms, C is -NH (CH₂)ₙCO- wherein n is 5 or 11; B is amino; A is alkylen having 6-14 C atoms optionally including up to 3 O atoms, and ma and mb which may be the same or different, is an integer 2-5.

Examples of preferred lubricants to be used in the iron based compositions according to the present invention are:
CH₃(CH₂)₁₆CO-[HN(CH₂)₁₁CO]₂-HN(CH₂)₁₂NH-[OC(CH₂)₁₁NH]₂-OC(CH₂)₁₆CH₃
CH₃(CH₂)₁₆CO-[HN(CH₂)₁₁CO]₂-HN(CH₂)₁₂NH-[OC(CH₂)₁₁NH]₃-OC(CH₂)₁₆CH₃
CH₃(CH₂)₁₆CO-[HN(CH₂)₁₁CO]₃-HN(CH₂)₁₂NH-[OC(CH₂)₁₁NH]₃-OC(CH₂)₁₆CH₃
CH₃(CH₂)₁₆CO-[HN(CH₂)₁₁CO]₃-HN(CH₂)₁₂NH-[OC(CH₂)₁₁NH]₄-OC(CH₂)₁₆CH₃
CH₃(CH₂)₁₆CO-[HN(CH₂)₁₁CO]₄-HN(CH₂)₁₂NH-[OC(CH₂)₁₁NH]₄-OC(CH₂)₁₆CH₃
CH₃(CH₂)₁₆CO-[HN(CH₂)₁₁CO]₄-HN(CH₂)₁₂NH-[OC(CH₂)₁₁NH]₅-OC(CH₂)₁₆CH₃
CH₃(CH₂)₁₆CO-[HN(CH₂)₁₁CO]₅-HN(CH₂)₁₂NH-[OC(CH₂)₁₁NH]₅-OC(CH₂)₁₆CH₃

Other examples are
CH₃)CO-HN(CH₂)₅CO-HN(CH₂)₂NH-OC(CH₂)₅NH-OC(CH₃) having the MW 370.49;
CH₃(CH₂)₂0CO-HN(CH₂)₁₁CO-HN(CH₂)₁₂NH-OC(CH₂)₁₁NH-OC(CH₂)₂₀CH₃ having the MW 1240.10
CH₃(CH₂)₂₀CO-[HN(CH₂)₁₁CO]₁₀-HN(CH₂)₁₂NH-[OC(CH₂)₁₁NH]₁₀-OC(CH₂)₂₀CH₃ having the MW 8738.04
CH₃(CH2)₄CO-[HN (CH₂)₁₁CO]₃-HN(CH₂)₁₂NH-[OC(CH₂)₁₁NH]₃-OC(CH₂)₄CH₃
having the MW 1580.53
CH₃(CH₂)₄CO-[HN(CH₂)₅CO]₇-HN(CH₂)₆NH-[OC(CH₂)₅NH]₇-OC(CH₂)₄CH₃ having the MW 1980.86
CH₃(CH₂)₂₀CO-[HN(CH₂)₅CO]₇-HN(CH₂)₆NH-[OC(CH₂)₅NH]₇-OC(CH₂)₂₀CH₃
having the MW 2429.69
and
CH₃(CH₂)₁₆NH-[OC(CH₂)₁₁NH]₄-CO(CH₂)₁₀CO-[HN(CH₂)₁₁CO]₄-HN (CH₂)₁₆CH₃
having the MW 2283.73

The chemical differences between the new lubricant and the lubricant described in the US patent 5,744,433 are that the new molecule has a central diamine or diacid moiety and identical terminal groups on both ends. The chemical difference between the new lubricant and the lubricant described in the US patent 5,154,881 is that the new lubricant molecule includes the unit -NH(CH)ₙCO-. In contrast to the lubricant known from US 5 154 881 no EBS is formed when the lubricant according to the present invention is prepared. EBS has the chemical formula CH₃(CH₂)₁₆CO-HN(CH₂)₂NH-OC(CH₂)₁₆CH₃) is a molecule without lactam units which is in contrast to the lubricants according to the present invention.

As regards the molecular weight of the new lubricant molecule it has been found that the preferred lubricants have a molecular weight between 1000 and 5000, most preferably between 1500 and 3000.

The lubricant molecule may be prepared according standard procedures for amide oligomer as described in e.g. "Principles of Polymerization" third edition by George Odian (John Wiley & Sons, Inc.). According to the present invention the lubricant preferably consists of at least 80% of the amide having the formula described above. Thus up to 20% by weight of other types of lubricants may be added, as long as the advantageous properties of the new lubricant is not detrimentally affected.

This lubricant, which is added to the iron-based powder is preferably in the form of a solid powder, can make up 0.1-1% by weight of the metal-powder composition, preferably 0.2-0.8% by weight, based on the total amount of the metal-powder composition. The possibility of using the lubricant according to the present invention in low amounts is an especially advantageous feature of the invention, since it enables high densities to be achieved.

As used in the description and the appended claims, the expression "iron-based powder" encompasses powder essentially made up of pure iron; iron powder that has been pre-alloyed with other substances improving the strength, the hardening properties, the electromagnetic properties or other desirable properties of the end products; and particles of iron mixed with particles of such alloying elements (diffusion annealed mixture or purely mechanical mixture). Examples of alloying elements are copper, molybdenum, chromium, manganese, phosphorus, carbon in the form of graphite, and tungsten, which are used either separately or in combination, e.g. in the form of compounds (Fe₃P and FeMo). Unexpectedly good results are obtained when the lubricants according to the invention are used in combination with iron-based powders having high compressibility. Generally, such powders have a low carbon content, preferably below 0.04% by weight. Such powders include e.g. Distaloy AE, Astaloy Mo and ASC 100.29, all of which are commercially available from Hoganas AB, Sweden.

Apart from the iron-based powder and the lubricant, the new powder composition may contain one or more additives such as binders, flow agents, processing aids and hard phases.

The binder may be added to the powder composition in accordance with the method described in U.S. Pat. No. 5,368,630 (which is hereby incorporated by reference) and may be organic compounds such as cellulose ester resins, hydroxyalkyl cellulose resins having 1-4 carbon atoms in the alkyl group, or thermoplastic phenolic resins.

A type of flow agent, which can be used according to the present invention, is disclosed in the US patent 5,782,954 (which is hereby incorporated by reference). The flow agent, which is preferably a silicon dioxide, is used in an amount from about 0.005 to about 2 percent by weight, preferably from about 0.01 to about 1 percent by weight, and more preferably from about 0.025 to about 0.5 percent by weight, based on the total weight of the metallurgical composition. Furthermore, the flow agent should have an average particle size below about 40 nanometers. Preferred silicon oxides are the silicon dioxide materials, both hydrophilic and hydrophobic forms, commercially available as the Aerosil line of silicon dioxides, such as the Aerosil 200 and R812 products, from Degussa Corporation.

The processing aids used in the metal-powder composition may consist of talc, forsterite, manganese sulphide, sulphur, molybdenum disulphide, boron nitride, tellurium, selenium, barium difluoride and calcium difluoride, which are used either separately or in combination.

The hard phases used in the metal-powder composition may consist of carbides of tungsten, vanadium, titanium, niobium, chromium, molybdenum, tantalum and zirconium, nitrides of aluminium, titanium, vanadium, molybdenum and chromium, Al₂ O₃, and various ceramic materials.

The invention is further illustrated by the following examples, which are to be interpreted only as examples but should not limit the scope of protection.

### EXAMPLE 1

The following tables disclose a comparison of properties between components prepared from powder mixtures including the lubricant according to the present invention and the amide type lubricant disclosed in the US patent 5,744, 433.

**Table 1**

| Lubricant | Compaction Pressure (MPa) | GD (g/cm³) | Ejection Force (N/mm²) | Ejection Energy (J/cm²) | Springback (%) |
|---|---|---|---|---|---|
| | | | | | |
| Invention | 500 | 7.14 | 11.5 | 19.3 | 0.147 |
| " | 600 | 7.29 | 11.4 | 23.3 | 0.162 |
| " | 700 | 7.38 | 11.8 | 24.6 | 0.192 |
| | | | | | |
| Orgasol 3501* | 500 | 7.09 | 11.9 | 29.9 | 0.191 |
| | 600 | 7.22 | 13.8 | 40.0 | 0.187 |
| | 700 | 7.30 | 16.0 | 48.5 | 0.229 |

**Table 2**

| Lubricant | Compaction Pressure (MPa) | Appearance | |
|---|---|---|---|
| | | Green compact | Die Wall |
| Invention | 500 | No stains | No deposit |
| " | 600 | Few stains | No deposit |
| " | 700 | Few stains | No deposit |
| | | | |
| Orgasol 3501* | 500 | Many stains | Some deposit |
| | 600 | Many stains | More deposit |
| | 700 | Many stains | More deposit |

| | | | |
|---|---|---|---|
| Temperature Powder/Die: 120°C/120°C * lubricant preferred according to US patent 5,744, 433 | | | |

The iron-based powder was Distaloy AE available from Höganäs AB, Sweden. This powder was mixed with 0.3% by weight of ultrafine graphite and 0.6% by weight of a lubricant according to the present invention. A flow enhancing agent Aerosil® 200 was added in an amount of 0.06% by weight.

As can be seen the new oligomer amide type lubricant according to the present invention is superior not only as regards the ejection force, the ejection energy, the springback but also when it comes to the appearance of the compacted component. Additionally the lubricant does not deposit on the die wall.

### EXAMPLE 2

The following table discloses a comparison of properties between components prepared from powder mixtures including the lubricant according to the present invention and the amide type lubricant disclosed in the US patent 5,154,881.

As can be seen the lubricant according to the present invention is superior as regards the ejection force, the ejection energy and the springback.

**Table 3**

| | GD (g/cm³) | Ejection Force (N/mm²) | Ejection Energy (J/cm²) | Springback (%) |
|---|---|---|---|---|
| Lubricant according to the present invention | 7.46 | 9.7 | 20.9 | 0.121 |
| Lubricant according to US patent 5 154 881 | 7.40 | 15.4 | 21.9 | 0.201 |
| Compaction pressure 700 MPa | | | | |
| Temperature powder/Die 130°C/150°C | | | | |

The iron-based powder was Distaloy AE available from Höganäs AB, Sweden.

This powder was mixed with 0.3% by weight of ultrafine graphite and 0.6% by weight of a lubricant according to the present invention. A flow enhancing agent Aerosil was added in an amount of 0.06% by weight.

### EXAMPLE 3

The following example discloses a comparison of densities of green bodies obtained with the oligomer amide lubricants which are used according to the present invention and which have different molecular weights.

The iron-based powder was Distaloy AE available from Höganäs AB, Sweden.

This powder was mixed with 0.3% by weight of ultrafine graphite and 0.6% by weight of a lubricant according to the present invention. A flow enhancing agent Aerosil was added in an amount of 0.06% by weight.

The powder was heated to a temperature of 130°C and the temperature of die was 150°C. The compaction pressure was 700 MPa.

| Molecular Weight of Lubricant | GD (g/cm³) |
|---|---|
| 2000 | 7,44 |
| 3000 | 7,41 |
| 4000 | 7,31 |

If the molecular weight of the oligomer amide lubricant is lower than (about) 2000 the properties of the powder composition becomes worse with regards to flow, and the lubricant will have a tendency of sticking to the die wall and the surface of the ejected compact. The sticky nature of such surfaces increases the risk of formation of rough surfaces on the final part owing to powder which may be collected onto the ejected compact.

## Claims

1. A powder composition for warm compaction comprising an iron-based powder and a lubricant powder, said lubricant consisting essentially of an amide represented by the following formula
D-Cₘₐ-B-A-B-C_{mb}-D
wherein
D is -H, COR, CNHR, wherein R is a straight or branched aliphatic or aromatic group including 2-21 C atoms
C is the group -NH (CH₂)ₙCO-
B is amino or carbonyl
A is alkylen having 4-16 C atoms optionally including up to 4 O atoms
ma is an integer 1-10
mb is an integer 1-10
n is an integer 5-11.

2. A powder composition according to claim 1 wherein D is COR, wherein R is an aliphatic group 16 - 20 C atoms, C is -NH (CH₂)ₙCO- wherein n is 5 or 11; B is amino; A is alkylen having 6-14 C atoms optionally including up to 3 O atoms, and ma and mb, respectively is an integer 2-5, whereby ma and mb may be the same or different.

3. A powder composition according to any one of the claims 1-2 wherein the lubricant consists of a compound selected from the group consisting of
CH₃(CH₂)₁₆CO-[HN(CH₂)₁₁CO]₂-HN(CH₂)₁₂NH-[OC(CH₂)₁₁NH]₂-OC(CH₂)₁₆CH₃
CH₃(CH₂)₁₆CO-[HN(CH₂)₁₁CO]₂-HN(CH₂)₁₂NH-[OC(CH₂)₁₁NH]₃-OC(CH₂)₁₆CH₃
CH₃(CH₂)₁₆CO-[HN(CH₂)₁₁CO]₃-HN(CH₂)₁₂NH-[OC(CH₂)₁₁NH]₃-OCCH₂)₁₆CH₃
CH₃(CH₂)₁₆CO-[HN(CH₂)₁₁CO]₃-HN(CH₂)₁₂NH-[OC(CH₂)₁₁NH]₄-OC(CH₂)₁₆CH₃
CH₃(CH₂)₁₆CO-[HN(CH₂)₁₁CO]₄-HN(CH₂)₁₂NH-[OC(CH₂)₁₁NH]₄-OC(CH₂)₁₆CH₃
CH₃(CH₂)₁₆CO-[HN(CH₂)₁₁CO]₄-HN(CH₂)₁₂NH-[OC(CH₂)₁₁NH]₅-OC(CH₂)₁₆CH₃
CH₃(CH₂)₁₆CO-[HN(CH₂)₁₁CO]₅-HN(CH₂)₁₂NH-[OC(CH₂)₁₁NH]₅-OC(CH₂)₁₆CH₃

4. A powder composition according to any one of the claims 1-3, wherein said amide has a molecular weight of 1500 to 3000 and is present in said composition in an amount of less than 1% by weight.

5. A powder composition according to any one of the claims 1-4, wherein the lubricant powder is provided in a concentration 0.2 to 0.8% by weight of the composition.

6. A powder composition according to any one of the claims 1-5, which additionally contains one or more additives selected from the group consisting of binders, processing aids, and hard phases.

7. A powder composition according to any one of the claims 1-6, wherein said iron-based powder is compressible, and at least 80% by weight of said lubricant powder is made up of said amide oligomer.

8. A powder composition according to any one of the claims 1-6, wherein said composition is essentially free from ethylenebisstearamide.

9. A powder composition according to any one of the claims 1-8, **characterised in that** said iron-based powder has a carbon content of at most 0.04% by weight.

10. A method for producing sintered products comprising:
(a) mixing an iron-based powder with a lubricant powder as defined in the previous claims;
(b) preheating the metal-powder composition,
(c) compacting the metal-powder composition in a pre-heated tool, and optionally
(d) sintering the compacted metal-powder composition at a temperature above 1050° C to form a sintered product.

## Patentansprüche

1. Pulverzusammensetzung zur Warmverdichtung umfassend ein Pulver auf Eisenbasis und ein Schmiermittelpulver, wobei das Schmiermittel im wesentlichen aus einem Amid besteht, dargestellt durch die folgende Formel:
D-Cₘₐ-B-A-B-C_{mb}-D
wobei
D -H, COR, CNHR ist, wobei R eine gerade oder verzweigte aliphatische oder aromatische Gruppe ist, umfassend 2 - 21 C-Atome
C die Gruppe -NH (CH₂)ₙ CO- ist,
B Amino oder Carbonyl ist,
A Alkenyl mit 4 - 16 C-Atomen ist, gegebenenfalls umfassend bis zu 4 O-Atomen,
ma eine Zahl von 1 - 10 ist,
mb eine Zahl von 1 - 10 ist,
n eine Zahl von 5 - 11 ist.

2. Pulverzusammensetzung nach Anspruch 1, wobei D COR ist, wobei R eine aliphatische Gruppe mit 16 bis 20 C-Atomen ist, C -NH (CH₂)ₙ CO- ist, wobei n 5 oder 11 ist; B ein Amino ist; A Alkylen mit 6-14 C-Atomen ist, gegebenenfalls umfassend bis zu 3 O-Atomen, und ma und mb, jeweils eine Zahl von 2 - 5 sind, wobei ma und mb gleich oder voneinander verschieden sein können.

3. Pulverzusammensetzung nach einem der Ansprüche 1 - 2, wobei das Schmiermittel aus einer Verbindung besteht, gewählt aus der Gruppe bestehend aus
CH₃(CH₂)₁₆CO-[HN(CH₂)₁₁CO]₂-HN(CH₂)₁₂NH-[OC(CH₂)₁₁NH]₂-OC(CH₂)₁₆CH₃
CH₃(CH₂)₁₆CO-[HN(CH₂)₁₁CO]₂-HN(CH₂)₁₂NH-[OC(CH₂)₁₁NH]₃-OC(CH₂)₁₆CH₃
CH₃(CH₂)₁₆CO-[HN(CH₂)₁₁CO]₃-HN(CH₂)₁₂NH-[OC(CH₂)₁₁NH]₃-OC(CH₂)₁₆CH₃
CH₃(CH₂)₁₆CO-[HN(CH₂)₁₁CO]₃-HN(CH₂)₁₂NH-[OC(CH₂)₁₁NH]₄-OC(CH₂)₁₆CH₃
CH₃(CH₂)₁₆CO-[HN(CH₂)₁₁CO]₄-HN(CH₂)₁₂NH-[OC(CH₂)₁₁NH]₄-OC(CH₂)₁₆CH₃
CH₃(CH₂)₁₆CO-[HN(CH₂)₁₁CO]₄-HN(CH₂)₁₂NH-[OC(CH₂)₁₁NH]₅-OC(CH₂)₁₆CH₃
CH₃(CH₂)₁₆CO-[HN(CH₂)₁₁CO]₅-HN(CH₂)₁₂NH-[OC(CH₂)₁₁NH]₅-OC(CH₂)₁₆CH₃

4. Pulverzusammensetzung nach einem der Ansprüche 1 - 3, wobei das Amid ein Molekulargewicht von 1.500 bis 3.000 aufweist und in der Zusammensetzung in einer Menge mit weniger als 1 Gew.-% vorhanden ist.

5. Pulverzusammensetzung nach einem der Ansprüche 1 - 4, wobei das Schmiermittelpulver in einer Konzentration von 0,2 bis 0,8 Gew.-% der Zusammensetzung bereitgestellt ist.

6. Pulverzusammensetzung nach einem der Ansprüche 1 - 5, welche zusätzlich einen oder mehrere Zusatzstoffe enthält, gewählt aus der Gruppe bestehend aus Bindemitteln, Verarbeitungshilfen und harten Phasen.

7. Pulverzusammensetzung nach einem der Ansprüche 1 - 6, wobei das Eisenbasispulver verdichtbar ist, und wobei wenigstens 80 Gew.-% des Schmiermittelpulvers aus dem Amid-Oligomer bestehen.

8. Pulverzusammensetzung nach einem der Ansprüche 1 - 6, wobei die Zusammensetzung im wesentlichen kein Ethylenbisstearamid aufweist.

9. Pulverzusammensetzung nach einem der Ansprüche 1 - 8, **dadurch gekennzeichnet, dass** das Pulver auf Eisenbasis einen Kohlenstoffgehalt von höchstens 0,04 Gew.-% aufweist.

10. Verfahren zur Herstellung von Sintererzeugnissen umfassend:
(a) Mischen eines Pulvers auf Eisenbasis mit einem Schmiermittelpulver, wie in den vorangehenden Ansprüchen definiert;
(b) Vorwärmen der Metall-Pulver-Zusammensetzung;
(c) Verdichten der Metall-Pulver-Zusammensetzung in einem vorgewärmten Werkzeug, und gegebenenfalls
(d) Sintern der verdichteten Metall-Pulver-Zusammensetzung bei einer Temperatur von oberhalb 1.050°C, um ein Sintererzeugnis zu bilden.

## Revendications

1. Composition de poudre pour compactage à chaud comprenant une poudre à base de fer et une poudre de lubrifiant, ledit lubrifiant étant constitué essentiellement d'un amide représenté par la formule suivante
D-Cₘₐ-B-A-B-C_{mb}-D
dans laquelle
D représente un atome d'hydrogène, un groupe COR, un groupe CNHR, dans lesquels R représente un groupe aliphatique ou aromatique linéaire ou ramifié comprenant 2 à 21 atomes de carbone,
C représente le groupe -NH (CH₂)ₙ CO-,
B représente un groupe amino ou un groupe carbonyle,
A représente un groupe alkylène ayant 4 à 16 atomes de carbone contenant éventuellement jusqu'à 4 atomes d'oxygène,
ma représente un nombre entier de 1 à 10,
mb représente un nombre entier de 1 à 10,
n représente un nombre entier de 5 à 11.

2. Composition de poudre selon la revendication 1, dans laquelle D représente un groupe COR, dans lequel R représente un groupe aliphatique ayant 16 à 20 atomes de carbone, C représente un groupe -NH (CH₂)ₙ CO-, dans lequel n a pour valeur 5 ou 11 ; B représente un groupe amino ; A représente un groupe alkylène ayant 6 à 14 atomes de carbone, contenant éventuellement jusqu'à 3 atomes d'oxygène, et ma et mb représentent respectivement un nombre entier de 2 à 5, ma et mb pouvant être identiques ou différents.

3. Composition de poudre selon l'une quelconque des revendications 1 ou 2, dans laquelle le lubrifiant est constitué d'un composé choisi dans le groupe constitué de :
CH₃(CH₂)₁₆CO-[HN(CH₂)₁₁CO]₂-HN(CH₂)₁₂NH-[OC(CH₂)₁₁NH]₂-OC(CH₂)₁₆CH₃
CH₃(CH₂)₁₆CO-[HN(CH₂)₁₁CO]₂-HN(CH₂)₁₂NH-[OC(CH₂)₁₁NH]₃-OC(CH₂)₁₆CH₃
CH₃(CH₂)₁₆CO-[HN(CH₂)₁₁CO]₃-HN(CH₂)₁₂NH-[OC(CH₂)₁₁NH]₃-OCCH₂)₁₆CH₃
CH₃(CH₂)₁₆CO-[HN(CH₂)₁₁CO]₃-HN(CH₂)₁₂NH-[OC(CH₂)₁₁NH]₄-OC(CH₂)₁₆CH₃
CH₃(CH₂)₁₆CO-[HN(CH₂)₁₁CO]₄-HN(CH₂)₁₂NH-[OC(CH₂)₁₁NH]₄-OC(CH₂)₁₆CH₃
CH₃(CH₂)₁₆CO-[HN(CH₂)₁₁CO]₄-HN(CH₂)₁₂NH-[OC(CH₂)₁₁NH]₅-OC(CH₂)₁₆CH₃
CH₃(CH₂)₁₆CO-[HN(CN₂)₁₁CO]₅-HN(CH₂)₁₂NH-[OC(CH₂)₁₁NH]₅-OC(CH₂)₁₆CH₃

4. Composition de poudre selon l'une quelconque des revendications 1 à 3, dans laquelle ledit amide a un poids moléculaire de 1500 à 3000 et est présent dans ladite composition en une quantité inférieure à 1 % en poids.

5. Composition de poudre selon l'une quelconque des revendications 1 à 4, dans laquelle la poudre de lubrifiant est présente dans une concentration de 0,2 à 0,8 % en poids de la composition.

6. Composition de poudre selon l'une quelconque des revendications 1 à 5, qui contient en outre un ou plusieurs additifs choisis dans le groupe constitué de liants, d'adjuvants de mise en oeuvre et de phases dures.

7. Composition de poudre selon l'une quelconque des revendications 1 à 6, dans laquelle ladite poudre à base de fer est compressible, et au moins 80 % en poids de ladite poudre de lubrifiant sont constitués dudit oligomère d'amide.

8. Composition de poudre selon l'une quelconque des revendications 1 à 6, ladite composition étant essentiellement exempte d'éthylènebisstéaramide.

9. Composition de poudre selon l'une quelconque des revendications 1 à 8, **caractérisée en ce que** ladite poudre à base de fer possède une teneur en carbone maximum de 0,04 % en poids.

10. Procédé de production de produits frittés consistant à :
(a) mélanger une poudre à base de fer avec une poudre de lubrifiant selon les revendications précédentes ;
(b) préchauffer la composition de poudre métallique ;
(c) compacter la composition de poudre métallique dans un outil préchauffé, et éventuellement,
(d) fritter la composition de poudre métallique compactée à une température supérieure à 1050 °C pour former un produit fritté.
